

## UNITED STATES PATENT OFFICE.

WALTER BROADBRIDGE, EDWIN EDSER, AND WILLIAM WARWICK STENNING, OF LONDON, ENGLAND, ASSIGNEES TO MINERALS SEPARATION NORTH AMERICAN CORPORATION, OF NEW YORK, N. Y., A CORPORATION OF MARYLAND.

## PRODUCTION OF BRIQUETTES.

No Drawing. Original application filed August 17, 1920, Serial No. 404,106. Divided and this application filed May 17, 1923. Serial No. 339,695.

To all whom it may concern:

Be it known that we, WALTER BROADBRIDGE, EDWIN EDSER, and WILLIAM WARWICK STENNING, subjects of the King of England, and residents of the city of London, England, have invented certain new and useful Improvements in the Production of Briquettes, of which the following is a specification.

10. This invention relates to the production of briquettes, and is herein illustrated as applied to the production of coal briquettes, and with coal concentrated from impure coal, coal dumps and the like.

15. One of the problems in briquetting is to secure an efficient coating of the coal particles by the binding medium, such as pitch, tar, resin, and the like.

In the froth-flotation process of concentrating ores as disclosed in Patent No. 835,120, to Sulman, Picard and Ballot, of November 6th, 1906, and later patents, it is known that the methods therein used for agitating a pulp of ore and water with an added agent, such as oil, tar and the like, result in a very effective coating of certain mineral particles with the added agent, and an equally effective flocculation of the particles which become readily separable from water, and we have now discovered by experiment that when finely divided coal in suspension in water is subjected to similar types of agitation in the presence of a liquefied binding medium, the coal particles become readily and thoroughly coated and also flocculated.

20. A feature of this invention, therefore, lies in the making of briquettes from carbonized fuel, whether artificially or naturally carbonized, as coal, by a process wherein the powdered coal, suspended in water, is subjected to agitation with a binding medium whereby the coal particles are coated with the binding medium and flocculated so as to be readily separable from water.

Again, in the froth-flotation process of concentrating ores it was frequently found desirable to add to the aqueous pulp certain agents which facilitated the segregation of 25 the desired mineral particles. In the specification such agents are referred to as floc-

culating agents, and it may be desirable to employ such an agent. Further, it is desirable that such agent, if employed, should itself subsequently assist as a binding agent 55 in the briquetting.

A further feature of this invention, therefore, consists in the employment in the pulp, during the above described agitation, of a flocculating agent, such as slaked lime, which 60 assists in the flocculation and subsequent draining of the coated coal particles, and also acts as an auxiliary binding agent in briquetting.

Again, in the froth-flotation process of 65 ore concentration, the action of the air in causing flocculation and rendering the concentrate particles readily separable from water is known, and it is a feature of this invention that the agitation of the coal-water pulp with the binding agent is conducted with a greater or less degree of aeration, either by agitation affecting or accompanied by the introduction of air or by air-agitation. 70

75. One process of producing coal briquettes from impure coal, coal dumps and the like, according to this invention, consists in crushing the crude material, if necessary, subjecting it to concentration and flotation 80 with the addition of a liquid agent which affords or contains both a frothing agent and a binding medium, and with or without a flocculating agent, such as slaked lime, whereby the coal particles become coated 85 with the binding medium, flocculated and floated in the form of agglomerates supported by bubbles, while the gangue is not so floated, collecting and draining the agglomerates and making the moist coal concentrate into briquettes. 90

## Example.

In this test a slurry obtained from a bituminous coking coal, containing 17% of 95 ash, was used, 400 grammes being made into a 4:1 pulp with water in a slide machine; 5% of melted pitch was added and cresol at the rate of 1½ lbs. per ton of the crude slurry, and kerosene oil at the rate of 1½ 100 lbs. per ton of the crude slurry. The pitch-coated coal was floated in the form of ag-

glomerates supported by bubbles, removed, filtered, masticated, kneaded and briquetted, and a briquette was made as described above. The briquette was of excellent qualities and contained 7½% of ash.

In cases where it is desired to recover the coated coal as a float, it is preferred to employ an agitation apparatus of the subaeration type, such, for example, as are disclosed 10 in the patents to Arthur Howard Higgins and one of us, William Warwick Stenning, No. 1,155,815, to said Arthur Howard Higgins, No. 1,155,816, and to Thomas Mackellar Owen, No. 1,155,836, each dated October 5, 15 1915.

In any of the above described agitations, the aqueous pulp may be heated to any desired degree to assist in disseminating the binding medium over the surface of the 20 coal particles; and as the water is conveniently employed in closed circuit, its temperature can be kept up without much expense.

The result of all of the above described 25 agitations with binding medium present is to form flocculations which are in fact agglomerations. The agglomerations tend to free themselves from the water of the pulp and therefore a very low moisture content 30 is readily attainable and is much more readily attainable than in the case of both flotation concentrates from ore concentration:

The binding agents employed may be 35 melted pitch, tar, resin and the like, or admixtures thereof. The flocculating agents may be slaked lime, sodium silicate and the like, referred to as saline flocculating agents.

This application is a division of our 40 pending application Serial Number 404,106, filed August 17th, 1920.

What we claim as our invention and desire to secure by Letters Patent is:—

1. A process of making briquettes of purified material from impure material which 45 consists in subjecting the impure material in a suitably divided condition to flotation separation, with the addition of material acting as frothing agent and binding medium and with a flocculating agent whereby 50 selected particles become coated, flocculated and floated in the form of agglomerates supported by bubbles, while impurities are not so floated, collecting and draining the float, and forming briquettes from the 55 coated particles.

2. A process of making fuel briquettes from impure carbonized fuel which consists in subjecting the crude material in a suitably divided condition to concentration 60 by a flotation process with the addition of material acting as frothing agent and binding medium and with a saline flocculating agent, whereby carbonized particles become coated, flocculated, and floated in the form 65 of agglomerates supported by bubbles, while

gangue is not so floated, collecting and draining the float, and forming briquettes from the coated particles.

3. A process of making briquettes of carbonized fuel which consists in agitating the 70 impure carbonized fuel in suitably divided condition in a freely flowing pulp with material acting as frothing agent and binding medium so as to coat carbonized particles and agglomerate them and float agglomerates of carbonized particles, and separating the floating agglomerates from pulp liquid and forming the agglomerates into briquettes. 75

4. A process of making relatively dry agglomerates of purified carbonized fuel which 80 consists in agitating the impure carbonized fuel in suitably divided condition in a freely flowing pulp with material acting as frothing agent and binding medium so as to coat carbonized particles and agglomerate them 85 and float agglomerates of carbonized particles, and separating the floating agglomerates from pulp liquid.

5. A process of making briquettes of carbonized fuel which consists in agitating the 90 impure carbonized fuel in suitably divided condition in a freely flowing pulp, with material acting as frothing agent and binding medium in amount sufficient to cause carbonized particles to agglomerate but insufficient to flow on the surface of the particles after coating the same, so as to coat carbonized particles and agglomerate them and float agglomerates of carbonized particles, and separating the floating agglomerates 95 from pulp liquid and forming the agglomerates into briquettes. 100

6. A process of making relatively dry agglomerates of purified carbonized fuel which 105 consists in agitating the impure carbonized fuel in suitably divided condition in a freely flowing pulp, with material acting as frothing agent and binding medium in amount sufficient to cause carbonized particles to agglomerate but insufficient to flow on the surface of the particles after coating the same, so as to coat carbonized particles and agglomerate them and float agglomerates of carbonized particles, and separating the floating agglomerates from pulp liquid. 110 115

7. A process of making briquettes of carbonized fuel which consists in agitating the 120 impure carbonized fuel in suitably divided condition in a freely flowing pulp, with material acting as frothing agent and binding medium and containing a large proportion of heavy hydrocarbons, so as to coat carbonized particles and agglomerate them and float agglomerates of the particles, and separating the floating agglomerates from pulp liquid and forming the agglomerates into briquettes. 125

8. A process of making relatively dry agglomerates of purified carbonized fuel which 130 consists in agitating the impure carbonized

- fuel in suitably divided condition in a freely flowing pulp, with material acting as frothing agent and binding medium and containing a large proportion of heavy hydrocarbons, so as to coat carbonized particles and agglomerate them and float agglomerates of the particles, and separating the floating agglomerates from pulp liquid.
9. A process of making briquettes of carbonized fuel which consists in agitating the impure carbonized fuel in suitably divided condition in a freely flowing pulp, with a sufficient amount of material acting as frothing agent and binding medium and containing a large proportion of heavy hydrocarbons to cause carbonized particles to agglomerate but insufficient to flow on the surface of the particles after coating the same, so as to coat carbonized particles and agglomerate them and float agglomerates of the particles, and separating the floating agglomerates from pulp liquid and forming the agglomerates into briquettes.
10. A process of making relatively dry agglomerates of purified carbonized fuel which consists in agitating the impure carbonized fuel in suitably divided condition in a freely flowing pulp, with a sufficient amount of material acting as frothing agent and binding medium and containing a large proportion of heavy hydrocarbons to cause carbonized particles to agglomerate but insufficient to flow on the surface of the particles after coating the same, so as to coat
- carbonized particles and agglomerate them and float agglomerates of the particles, and separating the floating agglomerates from pulp liquid.
11. A process of making briquettes of carbonized fuel which consists in agitating the impure carbonized fuel in suitably divided condition in a freely flowing pulp with material affording a frothing agent and containing pitch so as to coat carbonized particles and agglomerate them and float agglomerates of the particles, and separating the floating agglomerates from pulp liquid and forming the agglomerates into briquettes.
12. A process of making briquettes of carbonized fuel which consists in agitating the impure carbonized fuel in suitably divided condition in a freely flowing pulp, with a sufficient amount of material affording a frothing agent and containing pitch to cause carbonized particles to agglomerate but insufficient to flow on the surface of the particles after coating the same, so as to coat carbonized particles and agglomerate them and float agglomerates of the particles, and separating the floating agglomerates from pulp liquid and forming the agglomerates into briquettes.

In testimony whereof, we have affixed our signatures to this specification.

WALTER BROADBRIDGE.

EDWIN EDSER.

WILLIAM WARWICK STENNING.